

# UNITED STATES PATENT OFFICE.

SAMUEL LIPSIUS, OF NEW YORK, N. Y.

## PROCESS OF RAISING PRINTING.

1,158,065.

Specification of Letters Patent.

Patented Oct. 26, 1915.

No Drawing. Original application filed November 25, 1914, Serial No. 873,946. Divided and this application filed April 10, 1915. Serial No. 20,390.

To all whom it may concern:

Be it known that I, SAMUEL LIPSIUS, a citizen of the United States, and residing at New York, in the county of New York and State of New York, have invented a new and Improved Process of Raising Printing, of which the following specification is a full disclosure.

This application is a division of my co-pending case Ser. No. 873,946 filed Nov. 25, 1914, and the invention thereof relates to the printing of characters in simulation of the raised effects produced by the action of dies or engraved plates and ordinarily known as embossing work.

Various methods have heretofore been proposed and to some extent put into commercial use whereby embossed work may be simulated by acting in conjunction with an ordinary printing press, and without necessitating the manufacture of special dies. In practising these well-known methods, ordinary stiff, quick-drying printers' ink is first impressed upon a sheet of paper, a quantity of fusible resinous powder (such as gum elemi) is then deposited on the freshly inked surface and, by carefully melting this powder, it is caused to amalgamate with the inked surface so that when cold it will give a raised surface imitating the relief effects yielded by a die. This process has, however, possessed many heretofore unavoidable difficulties which have materially contributed to reduce the commercial value of the process. One difficulty with this imitation embossing, as heretofore practised, lies in the fact that the finished work has a very strong tendency to peel or strip on the paper so that, when the paper is folded or creased, the raised material will crack and flake, and the detached particles thereof will not only give the appearance of loose dirt scattered over the paper and collected in the folds thereof, but the neat effect of the printing itself is also lost. This has deprived this process of the very point on which its commercial utility depends: *i. e.*, a neatness and beauty comparable with die work.

Now one object within the contemplation of this invention is to create an improved process such as will yield a sheet of paper having printed characters not only closely imitating embossing but also so flexible and

so tenaciously adhering to the paper that it 55 may be folded without unduly cracking or flaking, so that the letter-heads on high grade bond paper may be folded or handled severely without a depreciation in appearance. 60

Another object is to render commercially available at a comparatively low cost a sheet of paper having raised characters characterized by a materially greater degree of flexibility than those produced by former methods 65 and characterized by a tenacity of adhesion to the paper which will enable them to remain intact on the paper notwithstanding considerable rough handling and folding.

Another object of this invention is to discover mutually compatible materials and the manner of utilizing the same, whereby the ultimate composition of the raised character will possess a considerable amount of elasticity or flexibility combined with a 75 strong tenacity for the paper so that the resultant printed matter may be given more durability.

A still further object is to create a method whereby, immediately after leaving the final 80 or hardening step, the raised printing will acquire a durable status on the paper so that the latter may at once be folded or handled without fear of producing flaking or the like.

Other objects will be indicated in connection with the following analysis of this invention which consists in the materials, the unique relations of the ingredients, the relative proportioning thereof, the method of 90 combining the same, and the resultant article of manufacture, all as more completely outlined herein.

To enable others skilled in the art so fully to comprehend the underlying features 95 thereof that they may embody the same by any of the numerous modifications in composition and method contemplated by this invention, the following description will outline the principles and rules to be observed. 100

As a result of exhaustive experiments, I have discovered and am enabled to cure two primary difficulties in the prevailing methods of imitating embossed work. That is to 105 say, I have found first, that by employing proper ingredients the ultimate composition of the raised characters will be compara-

tively flexible instead of being hard and brittle, and second that the composition may be caused to adhere much more tenaciously to the paper than is the case with the current methods. In the prevailing methods, the base of the character is first laid by blending it with ordinary stiff printers'-ink. By ordinary printers'-ink is meant an ink of the general type represented by the following formula or variations thereof, to wit: 68% heavy linseed oil varnish, 7% Japan drier, 19% carbon black, and 6% Prussian blue. On this quick-drying base is then applied the usual resinous composition, which is subsequently fused in place. Heretofore, it has not been observed that an incompatibility subsists between the ordinary printers'-ink and the resinous material used, under the conditions in which they are blended, and as a consequence the ultimate printed character has not been perfectly composed or constituted.

I have discovered that, by selecting an ink free from certain of the conventional ingredients and physical characteristics of ordinary stiff printing ink, and by selecting a compatible composition, and by properly blending the same, that an entirely different character is obtained which is at once comparatively flexible and which will adhere most tenaciously to the paper.

I have found that certain ingredients characteristically composing ordinary printers'-ink exercise a harmful effect. That is to say, ordinary stiff printers'-ink, among other things, contains material quantities of "drying" and of strong varnish-producing ingredients so that, from a theoretical aspect, ordinary printers'-ink may simply be regarded as a sort of quick-drying varnish. The reason for this lies in the fact that for all ordinary purposes it is highly desirable for the ink to take the form of a hard film almost immediately after leaving press so that it will not "offset" or "smudge" during subsequent manipulations. This immediate "set" is obtained by the agency of varnish-producing and "drying" ingredients and, in fact, a typical varnish is sometimes added to the other ingredients in making the ink. For example, a typical printing ink would more or less closely conform to the above-mentioned formula. My experiments have demonstrated, however, that the drying and varnish producing ingredients so desirable for ordinary stiff printers'-ink exercises a harmful effect when it is attempted to manipulate a printed character with the reliefing or embossing compound. That is to say, these ingredients are not sufficiently compatible with the fusible gum and they tend to impair the tenacity of adhesion and to render the gum brittle when applied to the paper. In practising this invention, the ink should contain a sufficient amount of oily

material, such as linseed oil or glycerin, to superficially penetrate the paper and amalgamate with the fusible gum, and the ink should possess greater fluidity than the ordinary tacky printers'-ink; *i.e.*, it should be sufficiently fluid almost to flow from its receptacle. An ink suitable for this purpose may be composed of 73% of boiled linseed oil, 8% of rosin, (as distinguished from a true drying agent), 12% of carbon black, 75 and 6% of Prussian blue. It will be observed that this formula is characteristically different from the constituents of ordinary printers'-ink and when it is used in connection with a suitable fusible gum, especially such as that hereinafter proposed, it will be found to be entirely compatible therewith and to produce a character that at once is flexible and yet adheres tenaciously to the paper immediately after leaving the printing press and melting oven. 85

My investigations have further developed a superior species of gum which will render much more satisfactory results than the gums heretofore employed with ordinary printers'-ink. That is to say, if ordinary shellac is freed from the limy, waxy substances and other foreign ingredients, so that substantially pure shellac or refined shellac is obtained, this product when powdered will be preëminently compatible with the typical ink above mentioned and it will, when fused in place, immediately after leaving the printing press, produce a character at once flexible and strongly adherent to the paper. 90

By using the ingredients herein specified and by completing the method immediately after leaving the printing press, it will be found that the cold sheets of printed matter may be stacked at once without danger of sticking together and they may be folded like an ordinary letter-head without chipping or flaking. 100

Without further analysis, the foregoing will so fully reveal the gist of this invention that others can by applying current knowledge readily adapt it for various applications without omitting certain features that, from the standpoint of the prior art, fairly constitute essential characteristics of the generic or specific aspects of this invention, and therefore such adaptations should and are intended to be comprehended within the meaning and range of equivalency of the following claims. 110

Having thus revealed this invention, I claim as new and desire to secure the following combinations of elements, or equivalents thereof, by Letters Patent of the United States:— 125

1. A process of the nature disclosed for producing raised printing, which comprehends printing a flat character by means of an ink containing boiled linseed oil; and 130

then fusing a gum of animal origin on said character.

2. A process of the nature disclosed for producing raised printing, which comprehends printing a flat character by means of an ink containing rosin and an oily agent, and then fusing a gum of animal origin on said character.

3. An article of manufacture consisting of a sheet of hard bond paper provided with printed characters raised in simulation of engraving and consisting of a fused compound composed of a shellac-like gum homogeneously blended into a water-free ink containing pigment but devoid of material amounts of quick-setting varnish elements; said characters adhering so tenaciously to the paper and being so flexible that said paper may be creased across said characters

without appreciably flaking and peeling said characters.

4. A process of producing raised flexible printing which comprehends imprinting on paper flat characters by means of a water-free ink containing oily material insoluble in water and pigment, but devoid of material amounts of quick-setting varnish elements, and then fusing onto said flat characters a powdered compound containing shellac.

In witness whereof, I hereunto subscribe my name, as attested by the two subscribing witnesses.

SAMUEL LIPSIUS.

Witnesses:

LEON MINTZ,  
B. COOKE.